

1

3,723,106

### MAGNETIC ALLOY

Juergen Schlenker, Parsippany, and Teh Po Wang, Cedar Grove, N.J., assignors to Wilbur B. Driver Co.  
No Drawing. Filed May 23, 1969, Ser. No. 827,180  
Int. Cl. C22c 19/00

U.S. Cl. 75—170

3 Claims

#### ABSTRACT OF THE DISCLOSURE

A magnetic alloy characterized by high permeability at low flux density and comprising, as expressed in percent by weight:

|            |           |
|------------|-----------|
| Molybdenum | 4.25—5.25 |
| Nickel     | 79—81     |
| Manganese  | 0.25—0.75 |
| Silicon    | 0.10—0.20 |
| Titanium   | 0.05—0.15 |
| Iron       | Balance   |

#### BACKGROUND OF THE INVENTION

Magnetic alloys known to the art as moly-permalloys are widely used as cores in transducers, transformers and the like. Characteristically, these alloys must exhibit high permeability at low flux density. This requirement is otherwise expressed as the necessity for these alloys to exhibit high initial permeability, which is defined as the ratio of increment magnetic flux density to incremental magnetizing force over a specified range of low values of flux density.

Recently, a demand has developed for magnetic alloys having values of initial permeability substantially higher than hitherto obtainable. We have succeeded in developing such alloys.

#### SUMMARY OF THE INVENTION

We have discovered that the additions of small amounts of silicon and titanium to our conventional moly-permalloy compositions results in substantially increased values of initial permeability.

In accordance with our invention, our magnetic alloy comprises, as expressed in percent by weight:

|            |           |
|------------|-----------|
| Nickel     | 79—81     |
| Molybdenum | 4.25—5.25 |
| Manganese  | 0.25—0.75 |
| Silicon    | 0.10—0.20 |
| Titanium   | 0.05—0.15 |
| Iron       | Balance   |

#### DETAILED DESCRIPTION OF PREFERRED EMBODIMENTS

One alloy composition in accordance with our invention is as follows:

|            | Percent |
|------------|---------|
| Nickel     | 79.66   |
| Molybdenum | 4.95    |
| Manganese  | 0.63    |
| Silicon    | 0.14    |
| Sulfur     | 0.001   |
| Titanium   | 0.10    |
| Carbon     | 0.003   |
| Iron       | Balance |

An ingot of the above composition was fabricated by conventional techniques and processed into 0.006 inch thick strip. Another ingot lacking silicon and titanium

2

but otherwise identical in composition was fabricated and processed in the same manner. This second composition is known and used by us. Samples from both strips were heated for four hours at 2150° F. in a hydrogen atmosphere. Thereafter, samples of both strips were subjected to a three-stage cooling process. The first stage utilizes the temperature range 2150° F. to 1100° F.; the second stage, the temperature range 1100° F.; and the third stage, the temperature range 600° F. to room temperature. The rates of cooling the first and third stages are not critical and do not influence initial permeability. The critical stage for cooling is the second stage which employs the temperature range of 1100° F. to 600° F. in which an ordering transformation occurs. Experimentally, we have determined that a rate of cooling of 375° F. per hour was optimum in this second stage and accordingly employed this rate in this second stage.

Four samples of each alloy composition were heat treated simultaneously in the same manner. The samples of our new alloy composition were found to have an average initial permeability, at forty gauss, of seventy two thousand gauss per oersted at a flux density of forty gauss. The samples of the known alloy composition were found to have an average initial permeability of forty thousand gauss per oersted at a flux density of forty gauss.

The magnetic characteristics outlined above can be maintained when the various constituents other than carbon and sulfur are maintained within the limits indicated. Carbon and sulphur are tramp elements and do not contribute by their presence to the characteristics desired. Indeed, excess quantities of carbon and sulfur can result in impaired magnetic properties. Thus the carbon content must not exceed 0.01% and the sulfur content must not exceed 0.005%.

What is claimed is:

1. A magnetic alloy characterized by high permeability at low flux density and consisting essentially of, as expressed in percent by weight:

|            |           |
|------------|-----------|
| Nickel     | 79—81     |
| Molybdenum | 4.25—5.25 |
| Manganese  | 0.25—0.75 |
| Silicon    | 0.10—0.20 |
| Titanium   | 0.05—0.15 |
| Iron       | Balance   |

2. An alloy as set forth in claim 1 having a specific composition as follows:

|            | Percent |
|------------|---------|
| Nickel     | 79.66   |
| Molybdenum | 4.95    |
| Manganese  | 0.63    |
| Silicon    | 0.14    |
| Titanium   | 0.10    |
| Iron       | Balance |

3. An alloy as set forth in claim 1 which also can contain up to 0.01% carbon and up to 0.005% sulfur.

#### References Cited

#### UNITED STATES PATENTS

3,269,834 8/1966 Lykens et al. 75—170

65 RICHARD O. DEAN, Primary Examiner

U.S. Cl. X.R.